

April 6, 1926.

1,579,889

F. REDDAWAY

BILLIARD TABLE CLOTH

Filed June 12, 1923

FIG. 1.

|   |   |   |   |   |   |   |   |   |   |    |    |    |
|---|---|---|---|---|---|---|---|---|---|----|----|----|
| 6 | X | X | X | X | X |   | X | X | X | X  | X  |    |
| 5 |   | X | X | X | X | X | X | X | X |    |    |    |
| 4 |   | X | X | X |   |   | X | X | X | X  | X  |    |
| 3 |   |   | X | X | X |   |   | X |   |    |    |    |
| 2 |   |   | X |   |   |   |   | X | X | X  |    |    |
| 1 |   |   |   | X |   |   |   |   | X |    |    |    |
|   | 1 | 2 | 3 | 4 | 5 | 6 | 7 | 8 | 9 | 10 | 11 | 12 |

FIG. 2



INVENTOR:

By *Frank Reddaway*  
*Wm Wallace White*  
ATTY.

## UNITED STATES PATENT OFFICE.

FRANK REDDAWAY, OF MANCHESTER, ENGLAND.

## BILLIARD-TABLE CLOTH.

Application filed June 12, 1923. Serial No. 644,847.

*To all whom it may concern:*

Be it known that I, FRANK REDDAWAY, a subject of the King of Great Britain and Ireland, residing at Cheltenham Street, 5 Pendleton, Manchester, in the county of Lancaster, England, have invented new and useful Improvements in Billiard-Table Cloths, of which the following is a specification.

10 The invention has reference to the cloth used for covering billiard tables. The cloth at present employed for this purpose is a fine woolen cloth woven to a certain thickness with a carefully finished surface and 15 is very expensive.

Under my invention I weave a cloth which is admirably adapted for the purpose from cotton, and the finished product in many respects possesses advantages over the wool- 20 en cloth, besides being very much cheaper. For the purpose of my invention I employ cotton of very fine counts, say from 60 to 100 count yarns, although I do not confine myself precisely to such, and the yarn used 25 is twisted from such fine counts and may be cleaned and gassed. From such cotton yarn I weave a homogeneous multiple fabric of the desired thickness and which possesses the requisite elasticity and softness. Such a 30 fabric may be of 3 or more cloths according to the fineness of the count of the cotton yarn, and is woven to show a plain weave surface on both sides. For this purpose, weaving a fabric of three cloths, I may use 35 a six shaft loom, although the material can be woven by other mechanism, such as by using a dobby or other means for conveniently operating the warp threads.

The accompanying diagram shows in Fig. 40 1 the "tie-up" in a six shaft loom, 12 to the round, suitable for weaving the improved cloth, and, Fig. 2 is a diagram showing the weft threads *a* in section.

The material when finished and dyed an 45 appropriate green colour, is eminently suitable for covering billiard tables and cushions. It is reversible, and possesses such a smooth surface that the ball will travel

faster than on an ordinary woolen billiard cloth. There is no nap to offer frictional 50 resistance to the travel of the ball, so that ironing is unnecessary, and the surface being very smooth offers no resistance to the cue tip, and thus is not liable to be accidentally 55 cut by the tip.

The method of manufacturing such new billiard table cloth from cotton may however be varied from that described, so that the result produces a homogeneous cloth of the requisite thickness, smoothness of surface, and elasticity.

I declare that what I claim is:

1. A reversible, napless cloth for covering billiard tables, comprising a homogeneous multiple fabric of a plurality of cloths solid woven in the loom from cotton yarns of fine counts doubled into the requisite number of folds and then twisted and gassed and dyed the appropriate color, said fabric being finished so as to produce a solid 70 woven, surfaced, napless, reversible cloth as herein described.

2. A napless, reversible cotton cloth for billiard tables, comprising a homogeneous multiple fabric of several cloths solid woven from cotton yarns of 60 to 100 counts doubled into the required number of folds and then twisted.

3. A napless, reversible cotton cloth for billiard tables, comprising a homogeneous, 80 multiple fabric of several cloths solid woven from cotton yarns of 60 to 100 counts doubled into the required number of folds and then twisted, said billiard cloth having a plain weave on both surfaces.

4. The process of producing a billiard cloth which consists in doubling cotton yarns of 60 to 100 counts into a plurality of folds, twisting the yarns, cleaning and gassing said yarns and weaving the same into a homogeneous, multiple, napless and reversible fabric.

In testimony whereof I have signed my name to this specification.

FRANK REDDAWAY.